

June 9, 1936.

W. E. McCULLOUGH

2,043,588

CADMUM COBALT BEARING ALLOY

Filed April 1, 1935

Fig. 1.



Fig. 2.



Fig. 3.



Inventor

WILLIAM E. McCULLOUGH

BY Whittmore, Hubert, Whittmore & Belknap

Attorneys

## UNITED STATES PATENT OFFICE

2,043,588

## CADMIUM-COBALT BEARING ALLOY

William E. McCullough, Detroit, Mich., assignor  
to Bohn Aluminum & Brass Corporation, De-  
troit, Mich., a corporation of Michigan

Application April 1, 1935, Serial No. 14,177

1 Claim. (Cl. 75—151)

The invention relates to bearing metal alloys and has for its object the obtaining of a material having novel and valuable characteristics. More particularly, it is an object to obtain a journal bearing which will stand up under high speed operation and without objectionable lapping or abrading action on the journal. In the present state of the art a type of bearing extensively used is one provided with a steel backing or shell and a lining of bearing metal. Among the essential characteristics of the bearing metal are, first, that it should form a firm bond with a steel shell or backing; second, that it should possess sufficient inherent strength to sustain the load; third, that its bearing surface should be free from any constituent which will cause an abrading or lapping action on the journal; fourth, that it should have a melting point sufficiently high to withstand the temperatures to which it is subjected in use. It is difficult to obtain any one material having all of these characteristics. Thus tin base babbitts are low in melting point and form a comparatively weak bond with the steel backing. Alloys having a cadmium base with a hardening constituent such as copper, magnesium or nickel form a stronger bond with the steel, but have a tendency to cause more or less lapping or abrasion of the journal. I have discovered that a cadmium base alloy using cobalt in place of copper or nickel as the hardening element has greatly improved properties, particularly in the absence of any tendency to lap or abrade the journals. The invention therefore consists in the cadmium cobalt alloy as hereinafter set forth.

35 In the drawing:

Fig. 1 illustrates a photomicrograph of my improved bearing material at a magnification of fifty diameters;

40 Figs. 2 and 3 are similar views at a magnification respectively of 100 and 500 diameters.

The specific alloy represented in the drawing is one containing 1.5% of cobalt and the balance cadmium. This exact proportion is not, however, essential for all uses, as I have discovered that 45 as high as 10% cobalt may be used for certain bearings and less than 1.5% in others.

The photomicrographs of the polished surface of this metal disclose a granular background in which is imbedded a constituent of needle-like ap-

pearance. It will also be noted that these needle-like elements traverse the grains at different angles.

Physical tests show changed properties which undoubtedly are due to this changed structure. 5 Thus at room temperature pure cadmium has a Brinell hardness of 21.5 whereas my improved cadmium cobalt alloy has a Brinell hardness of 31.2. Steel backed bearings lined with my cadmium cobalt alloy exhibit a uniformly tenacious 10 bond between the lining metal and the steel and when run against a steel journal of 200 Brinell gave the following test in comparison with babbitt lined bearings:

| Alloy         | A    |              |          | B    |              |          | C    |              |          |
|---------------|------|--------------|----------|------|--------------|----------|------|--------------|----------|
|               | Time | Load/Sq. In. | R. P. M. | Time | Load/Sq. In. | R. P. M. | Time | Load/Sq. In. | R. P. M. |
|               |      |              |          |      |              |          |      |              |          |
| Cd-Co-Babbitt | 2    | 1652         | 2948     | 2    | 2374         | 3500     | 6:45 | 3097         | 4070     |
| Dup....       | 2    | 1652         | 2948     | 2    | 2374         | 3500     | 0:50 | 3097         | 4070     |
|               | 2    | 1652         | 2948     | 2    | 2374         | 3500     | 1:40 | 3097         | 4070     |

From the foregoing it will be apparent that the cadmium cobalt alloy having the needle-like structure of hardening constituent, gives a bearing performance approximately five times better than that of a tin base babbitt when run under the same conditions, viz: bearing pressure 3097 30 pounds per square inch; R. P. M. 4070 on a journal of 2.125 diameter. It was also shown by these tests that the cadmium cobalt alloy has little tendency to lap the journal.

While I have described an alloy having only the two constituents, cadmium and cobalt, it is 40 obvious that other elements may be added to impart desired specific properties while still retaining the advantages of the cobalt cadmium combination.

45 What I claim as my invention is:

An alloy containing 1.5% to 10% of cobalt and the balance of cadmium.

WILLIAM E. McCULLOUGH. 50